

May 1, 1928.

1,667,721

L. G. COPEMAN

STONE MOLD

Filed May 29, 1925

2 Sheets-Sheet 1

*Fig. 1.*



*Fig. 2.*



*Fig. 3.*



*Fig. 4.*

INVENTOR:  
*Lloyd G. Copeman*  
BY  
*Stuart C. Barnes*  
ATTORNEY.

May 1, 1928.

1,667,721

L. G. COPEMAN

STONE MOLD

Filed May 29, 1925

2 Sheets-Sheet 2

Fig. 5



STONE

Fig. 6



Fig. 7



STONE

BY

INVENTOR:  
Lloyd G. Copeman  
Stuart C. Barnes  
ATTORNEY.

Patented May 1, 1928.

1,667,721

# UNITED STATES PATENT OFFICE.

LLOYD G. COPEMAN, OF FLINT, MICHIGAN, ASSIGNOR TO COPEMAN LABORATORIES COMPANY, OF FLINT, MICHIGAN, A CORPORATION OF MICHIGAN.

## STONE MOLD.

Application filed May 29, 1925. Serial No. 33,649

This invention relates to a pattern for forming a permanent impression of the pattern by which the patterns can be indeterminately reproduced at any time in 5 the future.

I am aware that it is not broadly new to take an impression of the pattern in plaster of Paris, but the impression thus made is a relatively soft, non-permanent impression 10 which cannot satisfactorily be stored for future reproductions of the pattern.

I have found that a mold section can be made of a composition employing about 20% magnesium oxide, by weight, 30% 15 finely ground silica, by weight, and 50% 50-mesh silica sand, by weight, and to which is added sufficient chloride of magnesium in solution at 26 Bé. specific gravity to form a mix which may be readily poured, and that 20 the resulting artificial stone has the property of neither expanding nor shrinking to any appreciable degree. This composition also solidifies into a permanent block of 25 artificial stone having relatively great hardness and resistance to wear, or fracture.

Of course a mold section made of a stone composition of this character, has utility wider than the molding of patterns, but it has its chief value as I now see it for this 30 purpose, as it permits the reproduction of patterns that are very accurate replicas of the master pattern, such as the wooden pattern which is first used to make the impression in the plastic stone.

In reproducing a mold block such as I have described one may proceed in several ways. For instance, if the parting line of the pattern is a straight one, one simply lays the flask section or drag on a flat surface, places the pattern in the flask and then 35 pours the composition which I have described, over the pattern. It may be desirable in order to prevent the wooden pattern sticking in the stone to utilize a stone pattern. This can be easily done by first 40 making an impression of the wooden pattern in a plaster cast and then casting a master pattern of this same stone mix in this plaster cast. This stone master pattern may then 45 be used to form the impression in the permanent mold block. It will be desirable, 50 however, before the pour is made into the flask to coat the stone pattern with a parting material. It will be found that such 55 a stone pattern separates from the permanent

stone block better than a wooden pattern, especially with the ordinary shellac coatings that are placed on these wooden patterns.

Where the pattern has an irregular parting line, the same is placed in a flask resting on a flat surface, and this is filled with sand with a suitable binding mix. The sand mix is then packed in about the pattern up to the parting line. Then the stone mix already described is poured in on this sand to fill the flask. When this hardened it will be obvious that one has a permanent block of stone which is a pattern impression. The other stone block, to form the opposite side of the pattern, can be easily cast by utilizing this first stone block by setting it in a flask, greasing or oiling the surface with any suitable parting material, the pattern itself being supported in the impression in this block and being coated with a parting material. Thereupon the remainder of the flask is filled up with the same mix, and when this is set one has a second artificial stone block with an impression of the other side of the pattern.

The molds may be coated with a very thin coating of waterproof material, or I may apply a thin coating of enamel, such for instance, as "Duco" or pyroxilin enamel.

I have illustrated the stone pattern block which is shown in its completed state in Fig. 1. In Fig. 2 the flask containing half the pattern, which has a straight parting line, is shown.

Fig. 3 shows the flask filled with the mix, which is allowed to set.

Fig. 4 shows the flask containing a pattern which has an irregular parting line and which is packed with sand.

Fig. 5 shows this sand flask with the stone poured in to form the mold block having the irregular parting line.

Fig. 6 shows the flask in which the first cast mold block, together with the pattern, is utilized to form the second mold block of stone.

Fig. 7 is a cross section taken on the line 7-7 of Fig. 6, with the pattern removed, showing the molds slightly separated.

What I claim is:

1. A permanent mold block for reproducing patterns, comprising an artificial stone block composed of cementitious composition employing silica, magnesium oxide,

and magnesium chloride, and in which is contained a permanent impression of at least a portion of the pattern to be cast.

2. A permanent mold section for casting and reproducing patterns, comprising a solid block of composition material containing substantially 20% of magnesium oxide, 30% of finely ground silica by weight, 50% of silica sand by weight, mixed with a solution of magnesium chloride, said block when hardened containing a permanent impression of a portion of a pattern.

3. A composition for making mold blocks comprising substantially 20% of magnesium oxide, 30% of silica, and 50% of silica sand mixed with a solution of magnesium chloride to the desired consistency.

4. A permanent mold block for reproducing patterns of a plastic material, comprising a block of artificial stone containing a permanent impression of at least a portion of the article to be reproduced, said artificial

stone being of a hard cementitious material of sufficient compressive strength to withstand the molding and removing of patterns and handling without chipping or breaking, whereby the same may be used for reproducing patterns at any time. 25

5. A composition for making mold blocks comprising substantially 20% of magnesium oxide, 30% of finely ground silica, and 50% of 50-mesh silica sand mixed with a solution of magnesium chloride in sufficient amount to give the desired consistency. 30

6. A composition for making mold blocks comprising substantially 20% of magnesium oxide, 30% of finely ground silica, and 50% of silica sand mixed to the desired consistency with a solution of magnesium chloride, having a specific gravity of 26 Bé. 35 40

In testimony whereof I have affixed my signature.

LLOYD G. COPEMAN.